

July 16, 1940.

F. G. BREYER

2,207,779

## PROCESS AND APPARATUS FOR ZINC SMELTING

Filed May 18, 1938

3 Sheets-Sheet 1



INVENTOR  
*FRANK G. BREYER*

BY  
*Hammond & Little*  
ATTORNEYS

July 16, 1940.

**F. G. BREYER**

2,207,779

## PROCESS AND APPARATUS FOR ZINC SMELTING

Filed May 18, 1938.

3 Sheets-Sheet 2



July 16, 1940.

**F. G. BREYER**

2,207,779

## PROCESS AND APPARATUS FOR ZINC SMELTING

Filed May 18, 1938

3 Sheets-Sheet 3



INVENTOR  
FRANK G. BREYER

BY

BY  
*Hammond & Lippold*  
ATTORNEYS

## UNITED STATES PATENT OFFICE

2,207,779

PROCESS AND APPARATUS FOR ZINC  
SMEILING

Frank G. Breyer, Wilton, Conn.

Application May 18, 1938, Serial No. 208,553

15 Claims. (CL. 75—87)

This invention relates to the production of metallic zinc by the smelting of the zinc-bearing raw materials.

The production of metallic zinc by pyrometallurgical processes up to a few years ago had invariably been accomplished by the use of relatively small gas-tight refractory retorts or muffles which extend directly into small individual condensers. The liberation of zinc as a vapor 5 from the solid residues in these retorts requires a reduction reaction at high temperature and with considerable absorption of heat. The heat necessary to sustain the reaction is generated by the combustion of fuel, like coal, coke or gas, 10 outside the retorts and conducted to the charges therein through the refractory retort walls. The condenser, luted into the front end of the retort and extending out of the heating zone into cooling air, is nothing more than a tapered 15 down prolongation of the retort, or zinc liberating chamber, and the zinc vapors generated in the retort move directly into the condenser where they are chilled and condensed to a pool of liquid zinc. A zinc furnace is a battery of these individual small retorts and condensers positioned 20 horizontally and enclosed in a fire brick setting and fired as a unit.

Each retort and its condenser of this conventional process constitute essentially a single 25 chamber or environment, and conditions in the condenser are controlled by conditions in the retort. Not only must sufficient heat to sustain the reduction reaction be conducted into the retort through its walls, but the fumes released in 30 the retort must be in a condensable condition so that when they reach the condenser and are chilled the zinc content may there condense out as a liquid pool of metal and be withdrawn from time to time manually.

One of the limitations of this conventional 35 process is that combustion or firing gases must be scrupulously excluded from the charge in a retort, since the admission of such gases results in the formation of blue powder or uncoalesced zinc particles in the condenser, instead of liquid zinc. For example, as soon as a zinc retort cracks 40 and fire gases penetrate into the charge the vapors will not condense and coalesce to liquid. In order to avoid wasting the zinc as oxide the 45 charge is promptly withdrawn from the retort when this occurs.

Another limitation of the usual process is that the nature of the charges supplied to the retorts must be carefully controlled, and retorts of very 50 small cross section accommodating correspond-

ingly small charges must be employed for satisfactory results. Zinc ores and reducing materials supplied to the retorts must be of high quality and of selected physical condition. There are many types of zinc-bearing materials which are not suitable. Moreover, the introduction of charges into the many retorts, their discharge, and the drawing of liquid zinc from the small condensers are burdensome operations which require a great deal of labor in the presence of 10 high temperatures, dust and fumes, which makes working conditions undesirable.

Still another disadvantageous feature of the conventional process is that the fuel requirements are very great because all of the CO generated 15 within the retort is burned in the air and lost and by far the larger portion of the heat generated by combustion around the retorts is wasted. Only a relatively small portion of the heat is conducted through the retort walls and into 20 the poorly heat-conducting residues for use in reacting the charge.

These limitations of the conventional zinc smelting process have long been recognized in the art, and various means have been tried with 25 the purpose of overcoming them. An improvement, which involves the use of vertical retorts developed by my co-workers and myself and described in United States Letters Patent Nos. 1,678,607, 1,680,726, 1,712,132, 1,712,133, 1,811,910, 30 1,832,354, and 1,832,356, has served to some extent to separate the furnace, which eliminates the zinc from the residues, from the condenser and to permit some degree of independent control of 35 these two stages of the process. This development, however, has by no means provided a satisfactory zinc smelting system, since the zinc releasing furnace must still produce zinc vapor in an environment from which combustion gases are excluded in order that the vapor may be condensed to liquid zinc when it reaches the condenser. This necessity still restricts the process to the use of retorts or muffles of relatively small 40 cross section and still subjects it to limiting raw material requirements, expensive preparation, 45 and wasteful methods of indirect heating.

If there is any one aspect of the problem that may be said to be dominant when smelting zinc by the use of equipment comparable in capacity to that used in lead and copper smelting, it is 50 the problem of conducting heat into a porous body of charge of any appreciable dimensions without the aid of rapidly moving fire gases. Using the charge as an electric resistor and thereby generating heat within the charge it- 55

self is a solution for certain types of ore, but it has not worked satisfactorily or economically on ores of low fusion point or low zinc content. On the other hand, if the heat could be generated by combustion of fuel in immediate and close contact with ore, the zinc could be eliminated from residues at a very rapid rate, as witness the very great tonnages of zinc eliminated from ore in a small space by the mechanical zinc oxide process. See article by Breyer in "The Mining Magazine," London, April, 1936. Rapid elimination of the zinc by direct firing would make possible furnace designs which, unhampered by the necessity of having muffle characteristics, would be capable of very great through-puts of bulky and poorly heat-conducting ores and residues. The production of zinc under such conditions, however, has not been accomplished by any process heretofore proposed.

20 An important object of my invention is to provide a new and improved process for zinc smelting which enables the liberation of zinc from residue by the reduction of zinc-bearing raw materials in the same chamber with combustible fuels and permits liquid metallic zinc to be recovered from the resulting mixture of zinc vapor, suspended zinc compounds and combustion gases.

Another object of the invention is to provide an improved zinc smelting process, and apparatus 30 for carrying out the same, which enable the handling of really large charges of zinc-bearing raw materials and fuels, permit the use of ores or other zinc-bearing materials of either low or high grade as well as cheaper fuels, reduce the labor requirements in zinc smelting and materially improve the conditions under which the operators of the process must work.

Another object of the invention is to provide a zinc smelting process involving several steps 40 which are carried out in independently controlled chambers so as to avoid limitations imposed on the zinc releasing and condensing operations by known processes.

Another object is to provide a process for producing both metallic zinc and zinc oxide as separate products by the fire reduction of the same charge of zinciferous raw material.

Another object is to provide a process for smelting zinc from raw material in which the heat of 50 reduction is supplied by combustion in the releasing chamber, and which produces gaseous products having a relatively high zinc content from which metallic zinc may be condensed.

Another object is to provide a zinc smelting 55 process in which zinc-bearing fumes are released from raw material in a chamber heated by internal combustion and the resulting fumes are subjected to rapid reduction and conditioned for effective condensation in a chamber controlled independently of the zinc releaser.

A further object of the invention is to provide a zinc smelting process comprising new and improved methods and means for efficiently extracting zinc values from dilute or rich gases containing 60 zinc vapor.

Another object of the invention is to provide new and improved apparatus for use in the smelting of zinc by the processes described and claimed herein.

70 Still another object of the invention is to provide a process which may be controlled and adapted for changing conditions of operation and for the production of metallic zinc from various types of zinciferous raw materials.

75 I have found that the foregoing and other de-

sirable features and advantages may be accomplished by an entirely new sequence of separately environed and controlled process steps and apparatus. I have discovered that the introduction of a fume conditioning furnace intermediate the zinc eliminator and the condenser permits the elimination of zinc from the raw material, on the one hand, and the condensation of the zinc, on the other, to be carried out independently in environments which are maintained under individual chemical, thermal and mechanical controls, and that the resulting freedom from limitations heretofore imposed upon zinc smelting operations may be utilized to modify the elimination step or the condensation step, or both, so that metallic zinc 10 may be produced practicably by elimination from ore or the like in a chamber where combustion occurs.

My process consists of three or more distinct stages which, though closely related to each other, are susceptible of a wide degree of variation and independent control. In the first stage I release zinc from zinciferous raw material in a furnace by the action of carbonaceous reducing material, the heat of reduction being supplied by combustion in the furnace chamber. The temperature in the furnace chamber preferably is kept in a relatively high range to influence the composition of the fumes favorably and to permit large outputs of products, and the operations incident to the elimination of the zinc preferably are controlled so as to obtain relatively large concentrations of zinc in the fumes issuing from the furnace. The charge is preheated to approximately 20 the reaction temperature before introduction into the chamber. The combustion-supporting gas preferably is preheated, and it may be enriched with oxygen in order to enhance the zinc content of the fumes. In a preferred embodiment I supply a large proportion of the heat necessary for 25 continuous reduction in the furnace by reoxidizing, or combusting, part of the zinc vapor and carbon monoxide which have previously been generated from the charge. It also is advantageous when using certain raw materials and 30 under certain conditions of operation to produce both metallic zinc and zinc oxide as separate products from the same charge material by treating the relatively rich fumes generated during 35 the early period of the reduction for the recovery 40 of metallic zinc according to my process, and thereafter burning to zinc oxide the more dilute fumes later generated.

The fumes generated in the first stage of the process contain variable amounts of zinc vapor, 45 carbon monoxide, carbon dioxide, nitrogen, and suspended reoxidized zinc. The content of carbon dioxide and reoxidized zinc depends largely upon the degree of reoxidation permitted in the furnace, and may vary from a small proportion 50 to a very large proportion when reoxidation is utilized as the principal source of heat for the reaction. These fumes, in a condition precluding 55 satisfactory condensation, are swept out of the furnace by pressure of the reaction products and are carried into a closed conditioning chamber containing a gas permeable charge of very hot, active reducing material, such as low temperature coke, lignite char or charcoal. The reducing 60 material has been preheated, deoxidized and degasified before being contacted by the fumes from the furnace. During the flow of fumes through 65 this material the influx of appreciable quantities of air or other gases, except from the eliminating 70 75

furnace, is prevented, and heat is supplied by means other than combustion within the chamber to sustain and complete the reduction of reducible constituents of the fumes in the gaseous or suspended form. The conditioning chamber provided for this purpose is of a size, appropriate to the capacity of the connected zinc eliminating furnace, which will subject the fumes passing therethrough to heating and reducing conditions for a period of time sufficient to effect substantially complete reduction of their content of  $\text{CO}_2$ ,  $\text{H}_2\text{O}$  and zinc oxide. Its charge of reducing material is kept readily pervious to the fumes so as to permit large through-puts and to avoid excessive pressure losses between the eliminating furnace and the condensers.

In this conditioning furnace, by the final reduction of oxidized materials in the fumes with or without other special treatments, fumes from which liquid zinc otherwise would not be obtainable are converted to a condensable condition. The treatment in the conditioner results in the delivery of completely reduced, dust-free vapors to the next stage of the process—the condensation stage. In addition, non-uniformities in the materials leaving the eliminating furnace can be treated variably and ironed out by suitable control of the conditioning chamber, which may be equipped to treat a variable supply and discharge a uniform exit product. In one embodiment of the process zinc waste material, such as zinc dross, zinc scrap, zinc die-castings and the like, may be redistilled by the sensible heat of the conditioned gases passing out of the chamber, resulting both in cooling the vapors for condensation and in enrichment of the vapor laden gases while going to the condensing apparatus. The gases leaving the conditioning chamber also may be subjected to treatment with sodium or other chlorides, or other surface fluxes or reducers of surface tension, in order to improve the coalescence. In still another embodiment, traces of sulfur and other substances which interfere with the condensation and the quality of the metal product may be removed by contacting the gases in the conditioning furnace with scrap iron, scrap copper or other "drag-downs," corresponding to "precipitants" in wet process purification process thereby eliminating impurities which otherwise would be condensed with or entrapped by the condensing zinc vapors.

The condensation of fully reduced, vapor laden gases leaving the conditioning furnace may be carried out in various types of condensers. When the gases are quite low in zinc vapor two condensers in series may be used to advantage—a liquid condenser and a powder condenser. In the liquid condenser, in addition to whatever cooling has occurred, e. g., through redistillation of zinc after reduction, the vapors are contacted with molten zinc metal to take advantage of the effects of evaporation. They are then cooled below the saturation point to collect the liquid product and thereafter preferably cooled rapidly in the powder condenser to deposit their residual zinc content as zinc dust, or blue powder. This powder may be returned to the upper part of the conditioning chamber to be redistilled by the sensible heat of the gases, enriching them to the point where a higher percentage of liquid is condensed and a lower percentage of powder. This system will ultimately come into equilibrium and all the metal will be recovered as liquid. When the gases in the powder condenser are

quite dilute and require a large loss of heat through its walls, I may cool these walls by air and subsequently use the hot air to combust fuel gases, when such are used to heat the conditioning furnace, or to blast the zinc eliminating furnace, or to preheat the solids going to either furnace.

By the use of the process described in general above I am able to release zinc from residue by any procedure best suited for the specific zinc raw material and the availability of fuels or electric power, as a relatively concentrated fume and without regard to the condensibility of the fumes as they leave the eliminating furnace. This process might be said to be a fire concentration of the zinc with subsequent reduction of the metal in gaseous suspension in a separate furnace. By its use all the advantages of fire concentration of zinc are to be had without the low heat economies and the collecting and handling and reworking costs of the ordinary process where the gases are cooled down and the zinc and other suspended matter separated and collected, densified and reworked in another furnace as a charge for metal or oxide.

The importance of the flexibility of my new process will be readily apparent to persons skilled in the art. Since the elimination of the zinc from the residue may take place in directly fired furnaces the problem of carrying heat economically into a bulk of porous ore and coal is solved. Only the final conditioning of the resulting fumes in the conditioning chamber need be accomplished by indirect or more expensive heating methods. In this conditioning chamber heat transfer is mostly to gases and solids in extremely fine suspension which, by their velocity, have high transfer rates and because they are extremely finely divided, reduce easily. The process is freed from other limitations which are inherent in the usual retort practice. Large charges of zinc-bearing raw materials, of almost any quality and physical condition, may be treated satisfactorily, and fuels of an inexpensive and readily accessible type may be used for combustion. Mechanical furnaces can be used which will handle one hundred tons or more of zinc charge per day, the fumes from which are passed through closely controlled conditioning columns for treatment therein and thence to communicating condensers where they condense to liquid zinc.

Other features and advantages of the invention will be made more apparent by the ensuing detailed description of illustrative embodiments when considered in connection with the accompanying drawings illustrating suitable apparatus which I have provided for practicing the invention. In the drawings,

Figure 1 is a front elevation, partly in section, of a complete zinc smelting assembly, including a zinc eliminating furnace, a conditioning chamber and a condensing system together with provision for producing zinc oxide from the same charge as used in the eliminating furnace.

Figure 2 shows an assembly of another form of apparatus which may be used instead of the apparatus shown in Figure 1.

Figure 3 is a view in vertical section of a special condensing system forming a part of the assembly illustrated in Figure 2.

Figure 4 shows another form of zinc eliminating furnace in combination with another form of conditioning furnace and a condenser.

In the practice of the invention by the use

of apparatus of the types illustrated in the several figures of the drawings, the elimination of zinc from residue is carried out in a furnace chamber designated generally by the character 5 A, and the furnace fumes from the zinc eliminating chamber A, including zinc and zinc compounds in suspension, pass to a conditioning chamber B where reducible constituents thereof are reduced and the fumes are conditioned for 10 condensation. From chamber B the zinc laden gases flow into condensation apparatus C where metallic zinc is recovered. Each of these stages of treatment is kept under individual control and adapted for best performance of the whole 15 under varying conditions of operation, as described in greater detail below.

In the practice of the invention according to one embodiment I may employ a modified traveling grate furnace such as illustrated in Figure 20 1 for the elimination of zinc from the residue. The furnace is composed of suitable refractory furnace walls 10 which define chambers within the furnace, separated by arches 29, and enclose a traveling grate upon which the charge of 25 zinc-bearing raw material, reducing materials and fuel is continuously fed. The grate 12 comprises a plurality of interconnected sections forming a continuous conveyor, the sections being made of heat-resisting material and spaced 30 to permit the passage of combustion-supporting gas therebetween but to prevent the sifting of briquetted material therethrough. This grate 12 passes over appropriate sprocket wheels 14 and 16, respectively, and beneath its upper flight air 35 boxes 18, 20, 22 and 24 are provided which extend across the furnace structure at appropriate intervals and serve to supply regulated streams of combustion-supporting gas, such as air, to the under side of the grate. The grate is arranged 40 to pass beneath hoppers 26 and 28, respectively, the former for briquetted fuel and the latter for briquettes of zinc-bearing raw material and carbonaceous reducing material. Intermediate 45 these hoppers the grate passes through a fuel ignition chamber 30. Beyond hopper 28 is an additional combustion chamber 32, for bringing the charge to a reaction temperature, and beyond this chamber are located larger, zinc eliminating chambers 33 and 34 in which combustion 50 and reduction of the charge take place. In the walls of the zinc eliminating chambers, above the grate, inlets for combustion-supporting gas are provided, for example as shown at 33a and 34a, for a purpose hereinafter described.

55 In the operation of the furnace, as the grate moves beneath hopper 26 a bed of fuel is fed onto the grate and then carried into the fuel ignition chamber 30 where it is ignited and from which combustion gases are withdrawn through 60 a suitable stack 36. The bed of ignited fuel is then carried beneath the hopper 28 for the charge materials, and briquettes of zinc-bearing raw material, such as zinciferous ore, and reducing material, such as coke, are fed into the ignited bed of fuel at this point. The layers of material are then carried into combustion chamber 32 where the entire charge is brought up to a 65 reaction temperature and from which gases are withdrawn through a stack 38. As the grate proceeds in its movement it then carries the ignited materials, at a reaction temperature, into the zinc eliminating chambers 33 and 34 where there occur continuous combustion, generation 70 of heat and continuous reduction of the zinc-

bearing raw material with consequent evolution of zinc-laden fumes.

In the preferred manner of eliminating the zinc at A in Figure 1, a relatively small volume of air or other combustion-supporting gas is 5 fed upwardly into the charge through the grate 12, enough to keep the grate relatively cool and to maintain active reduction in the lower portion 10 of the charge. The remaining oxygen necessary for combustion to keep the materials well above the reduction temperature is supplied by passing air or an oxygen-enriched gas, preferably preheated as high as practicable, into the chamber A at a point above the charge where part of the zinc vapor and carbon monoxide already generated 15 will be reoxidized to carbon dioxide and suspended particles of zinc oxide. In this manner the zinc content of the fumes leaving the furnace may be greatly increased as compared with a process in which the heat required for the reduction reaction is supplied substantially entirely by burning carbon. Assuming no heat losses and all of the reaction materials preheated to reaction temperature, the reduction would be maintained on a continuous basis, with no burning 20 of carbon, by reoxidizing less than half of the zinc vapor and carbon monoxide. In practice, when using the traveling grate type of eliminating furnace, a part of the heat necessary to sustain the reactions is supplied by the combustion of carbon and the remainder by combustion of zinc vapor and carbon monoxide, and fumes containing a relatively high proportion of zinc and zinc compounds are continuously discharged 25 from sections 33 and 34 of the zinc eliminating 30 chamber A through heat insulated off-takes 40 and 42. The fumes are carried by the respective off-takes into conditioning chambers B where further treatment takes place, as hereinafter described, in order to condition them for recovery 35 of their zinc content.

In addition to the zinc eliminating chamber A, the traveling grate furnace is conveniently provided with at least one chamber 35 located beyond the former and separated therefrom by an arch 45 29. For greatest efficiency in the metal production the charge on the grate 12 is kept in chambers 33 and 34 until the rate of reaction becomes retarded, which may occur after about three-fourths of the zinc content is exhausted, and it 50 then passes into chamber 35 where it is fired by an air blast from beneath the grate. The fumes from this chamber are then conveyed by an off-take 44 into a burner E for the production of zinc oxide. With this system the proportions of metallic zinc and zinc oxide produced from the 55 charge may be varied over a wide range, depending upon market conditions, etc., and requirements for both products may be supplied by the operation of the same furnace on the same raw 60 materials.

The fire reduction which takes place in the reduction chambers 33 and 34 is capable of utilizing various types of zinc residues and fuels as the raw materials and of producing large 65 volumes of fumes for the recovery of metallic zinc. The temperature in these chambers is kept in a high range to foster rapid reduction and the maintenance of pressures sufficient to drive the fumes through the other stages of the process. 70 A suitable balance of pressures between chambers 33 and 34 and adjacent chambers 32 and 35 can be effected by appropriate venting of the latter.

The conditioning apparatus used in the second 75

stage of the present process may be substantially the same regardless of whether a zinc eliminating furnace of the type illustrated in Figures 1, 2 and 4, or of other types, is used. It preferably comprises a column of granulated coke or other active carbonaceous reducing material heated to a temperature considerably above the reducing point of zinc oxide, carbon dioxide and water vapor and operated so that such compounds in the fumes entering the column are reduced substantially entirely and the resulting gases conditioned for effective condensation of liquid zinc in the condensation stage of the process. The carbonaceous reducing material is contained in a gas-tight chamber to which heat may be supplied either by burning fuel outside the chamber and transferring the heat through its walls or by making the column itself a resistor in an electric circuit and generating the required heat electrically within the chamber itself. Provision is made for feeding pre-heated and deoxidized coke at the top of the column and for removing reducing material at the bottom before its efficiency for conditioning the fumes has been substantially impaired. The column itself should provide considerable space for carrying out the reduction reactions, and its heating capacity should be ample so as to ensure thorough reduction of oxidized compounds in the fumes and to permit large through-puts of gases. The higher the temperatures maintained in the column the lower its volume may be per unit volume of fumes to be treated. When the coke is heated to approximately 1200° C. about 50 to 100 cubic feet of conditioner volume should be provided per 1000 cubic feet of exit gases per minute.

The conditioning chamber 46 is typical of one suitable construction using electricity for heating, and the chamber 200 in Figure 4 represents a suitable type of construction heated by external firing. In Figure 1, the chamber 46 has gas-tight walls including an outer metallic shell 52 and an inner layer of fire brick or other refractory material 54. Adjacent its top end it is formed with a restricted neck 56 which is normally kept closed by a rotatable gate valve 58 permitting the introduction of solid material into the chamber at will, but normally excluding air from the chamber. Through valve 58 the chamber communicates with a hopper 60 for the reception of conditioning material from a charging floor 62. The top of hopper 60 is usually covered by a movable gate 61 which may be moved to an open position to permit the introduction of material into the hopper from a car 64. The lower part of chamber 46 includes a restricted neck 66, also normally closed by a rotatable gate valve 68, through which material from the chamber may be discharged into a suitable receptacle on a floor 70. Since the fumes from the zinc eliminating furnace and off-take 40 pass upwardly through the chamber and the conditioning material is introduced into the chamber at the top, the described arrangement provides descending columns which result in efficient utilization of the material therein and enable easy adaptation of the rate of flow to requirements of the process.

Each conditioning chamber may include a bleeder 71 extending from the top portion of the chamber and controlled, for example, by a valve 71a for regulating the flow of gases therethrough. The purpose of the bleeder is to permit any oxidizing gases introduced into the top of the cham-

ber by the charge materials to be bled off, so that passage of such gases into the condensation apparatus with zinc laden gases may be avoided.

The heating means illustrated in Figure 1 includes an upper series of electrodes 72 extending into material in the chamber and a lower series of electrodes 74. With a column of coke in the chamber electrical current may be passed through these electrodes and through the coke to raise the temperature of the material to the proper point and to maintain such temperatures while fumes from the releasing furnace pass through the chamber. Heating the column in this way permits ready control over the temperatures and conditions of reaction therein. The heat required in the column is the heat generated by reoxidation in the eliminating furnace plus all losses which occur after the fumes leave the eliminator. Since the materials being reduced are composed of gases and very finely divided suspended compounds, reduction is very rapid, and heat transfer, whether from electrically heated coke or through the walls of the conditioning chamber, is efficient. The large through-puts of materials per unit volume of equipment and the freedom of selection of materials in the several stages of the process render operations economical and efficient in comparison with known smelting practices.

In addition to reducing material, such as coke, lignite, charcoal and activated carbon, I may introduce in like manner, controlled amounts of zinc scrap material, such as zinc dust, zinc-dross, zinc scrap, zinc die-castings and the like into the upper part of the conditioning chamber and redistill the same by means of the sensible heat of the previously reduced gases. I may also introduce "drag-downs" or condensation promoters as described hereinabove. These practices accelerate the subsequent condensation of molten zinc from the gases and at the same time purify the scrap materials introduced into the chamber.

From the conditioning chambers 46 and 48, whether of the type just described or of other types to be described below, completely reduced and conditioned zinc-laden gases pass outwardly through conduits 82 and 84 and thence into condensing apparatus C, which may be of any suitable construction or, when the gases are relatively lean in zinc vapor, preferably is adapted specially for efficient recovery of metallic zinc, for example, as illustrated in Figure 2 or 4.

In the embodiment shown in Figure 1, the condensing apparatus comprises chambers 76 and 78 having inside baffles which cause the gases to swirl through the chambers and to condense on the walls thereof and collect in a well or sump 88, whence liquid zinc may be withdrawn through a port 90 adjacent a floor level 92. The chambers are cooled, for example, by fins 79 or other cooling means. The residual gases from which zinc vapor has been condensed are withdrawn from the condensers through stacks 94 and 96 and then carried off for combustion uses or for other purposes, for example, in the conduit 99 which also receives combustion gases from chamber 32 of the travelling grate furnace.

It will be noted that conduits 40 and 42 from the zinc eliminating furnace enter the conditioning chambers 46 and 48 at a point where the entering fumes immediately contact very hot conditioning material. This is important to satisfactory operation, since it prevents chilling of the fumes, subjects them to conditioning treatment under the optimum circumstances, and

avoids loss of zinc values which otherwise might occur to an objectionable extent upon contact between the fumes and cooler material.

By use of the present process, I am able to release fumes from the metalliferous charge in the zinc eliminating furnace which include what have heretofore been considered objectionable combustion gases and to condition these fumes before they are introduced into the condensing apparatus so that they are no longer objectionable and so that an efficient recovery of liquid zinc is obtained. As already indicated, the process permits variations in the type of apparatus used in each stage. Several preferred variations are illustrated in Figures 2 to 4 of the drawings.

Figure 2 illustrates an assembly in which a blast furnace of the slagging type is used for the elimination of zinc from zinciferous ore and in which special condensing apparatus is employed to enhance the recovery of metallic zinc from relatively lean zinc-laden fumes. The eliminating furnace is designated 100 in Figure 2, and is constructed in a well known manner to provide a chamber A in which the reaction of a charge of fuel, ore and reducing material takes place. A hearth 102 is located at the bottom of the furnace chamber, and a well 104 communicates with the hearth for the collection of lead and matte when the ore contains lead and matte-forming material. A header 106 for a blast of combustion-supporting gas surrounds the furnace and is connected with a series of tuyères 108 for the introduction of a blast of air or other gas, preferably preheated, into the charge. Solid material forming the charge is dropped into the furnace chamber from a bin 110 through a restricted neck 112, controlled by a bell valve 114. The furnace gases containing the zinc leave the furnace chamber through a port 116 and a flue 118 connected with a conditioning chamber 120. The chamber 120 illustrated in Figure 2 is constructed like chambers 46 and 48 of Figure 1, although other types of conditioning apparatus may be used in its place. Conditioned fumes from the chamber 120 leave through a flue 156 adjacent the upper end of the chamber and thence pass to the condensing apparatus which is illustrated in greater detail in Figure 3.

The condensing apparatus illustrated in Figures 2 and 3 includes a liquid condenser and a powder condenser. Chamber C is a liquid zinc condenser similar to those shown in Figure 1. Chamber D is a zinc dust or blue powder condenser with large metal surface cooling areas 150 and ample baffling 152 to settle out the last of the zinc in the reduced gases. It is provided with conveying means, for example, a screw conveyor 154, at the bottom or hopper portion, so that the collected powder may be continuously or intermittently returned to the conditioning chamber for revolatilization by the sensible heat of the previously reduced gases. The conditioned gases from B enter C by way of the port and flue 156. Molten metal condenses out in C and may be tapped off from the tap hole 158. The partially condensed gases pass then into the blue powder condenser D where, due to the intense cooling, the last of the zinc is dropped out. The non-condensable gases of high fuel value leave this condenser through a flue 160 to be used for any suitable purpose, such as in the degassing and deoxidizing furnaces for the metalliferous charge and the conditioning chamber coke. I may also burn it in regenerators or recuperators to preheat the blast for the furnace A or use it

for indirectly heating the conditioning chamber B instead of the electric resistance method shown in Figure 2.

Charge materials introduced into the blast furnace 100 are preheated, degasified and freed of substances which readily oxidize zinc vapor before introduction into the combustion chamber of the furnace. The materials may be prepared in this manner by the use of apparatus communicating with the bin 110 including a hopper 130 for the reception of zinc bearing material, such as ore, and carbonaceous materials, such as coal, a kiln 132 for the preliminary treatment of these materials, a burner 134 and a conduit 136 connecting an end of kiln 132 with bin 110. The material in hopper 130 is fed to the kiln 132 through a conduit 138, the flow being controlled by a rotatable gate 140. Kiln 132 is mounted for rotation about its longitudinal axis, as by a sprocket chain 142 passing over a sprocket 144 surrounding the kiln. In this manner the solid materials passing through the kiln are kept in a state of agitation, and preliminary deoxidation and degasification thereof are facilitated. Burner 134 extends axially into the kiln through one of its ends so that solid materials approaching the burner are thoroughly treated before they leave the kiln through conduit 136. Gases from the kiln pass off through a waste stack 146. Solid materials entering conduit 136 are conveyed into bin 110, for example, by a screw conveyor 148. By the use of apparatus of this type a suitably proportioned mixture of deoxidized, degasified and preheated ore and carbonaceous material may be introduced into bin 110 at the desired rate, and from bin 110 these materials may be charged into the furnace chamber through restricted neck 112 simply by lowering the bell valve 114. The conditioning material fed into chambers B may be degasified, deoxidized and preheated and then fed to these chambers by similar apparatus.

As fuel for burner 134, I may use powdered coal, oil or gaseous fuels, but I prefer to use residual gases taken off from the condensation stage of the process because of the economic advantage thus obtained. It will be understood that burner 134 may communicate in any suitable manner with a gas take-off from a condensing apparatus, such as the take-off 160 illustrated in Figure 3 of the drawings.

A further assembly of apparatus suitable for use in the improved process is illustrated in Figure 4. The zinc eliminating chamber A in this figure is the furnace of the Waelz kiln type, including an elongated tube 300 that connects with suitable headers 302 and 304 at each end and is mounted for rotation around its longitudinal axis. One end of the kiln is positioned at a higher elevation than the other end so that solid charge materials introduced thereto move gradually along the length of the kiln as it rotates. The kiln is usually supported on spaced rotatable bearings such as indicated at 306 and 308 and is rotated by driving means such as a ring gear 310 surrounding the outside of the kiln and a driven pinion 312 meshing therewith. Various means may be used for supplying a preheated charge including zinciferous and carbonaceous reducing materials and fuel into the entry end of the kiln, for example, through a delivery chute 314. Adjacent the lower end of the kiln the header 304 is equipped with means 316 for introducing combustion-supporting gas, preferably highly heated air, into the furnace, 75

and with a well or receptacle 318 for receiving the reacted materials after they have traversed the length of the kiln. The header 302 communicates with an exit 320 which carries zinc-bearing gases from the furnace chamber to a conditioning chamber B, which in this embodiment is provided by an indirectly fired vertical retort 200.

The Waelz-type kiln is advantageous for use in the economical elimination of zinc from raw materials of low grade. In operation, an inclination and rate of rotation of the kiln are adopted which subject the charge to reaction conditions for a considerable period of time. The constant revolution of the kiln maintains a degree of agitation and mixing of the constituents of the charge which promotes a high elimination of their zinc content. The heat and blast requirements of this type of operation are relatively low because of its adaptability for the reoxidation of a large proportion of the zinc vapor and carbon monoxide initially liberated from the charge before the gases leave the furnace, so that the endothermic heat requirements of the reduction reaction are substantially compensated by the exothermic reoxidation of the zinc and carbon monoxide. The operation of this apparatus thus produces gases of relatively high zinc content, and the condition of the gases is such that they may be passed through a conditioning chamber B in accordance with my invention and there contacted with reducing material while heat is supplied so as to convert them to a condensable condition.

The conditioning furnace illustrated in Figure 4 comprises a vertical retort 200, similar to the conventional vertical coke retort, which includes one or more conditioning chambers B and is heated indirectly by the combustion of gases. A column 202 of coke or other reducing material is maintained within chamber B, degassed and deoxidized reducing material being fed into the chamber through an overlying hopper 204, for example as in Figure 2. A valve-controlled bleeder 71 may communicate with the top portion of the furnace, described in connection with Fig. 1 for the purpose. Used and dirty reducing material is withdrawn from the furnace from time to time through the sealed valve 206 at the bottom thereof. Combustion flues 208 extend vertically adjacent the walls of chamber B so that heat generated in the flues by combustion may be transmitted efficiently into the charge. Flues 208 communicate with upper and lower conduits 210 and 212 which supply suitable gaseous fuel taken from a pipe 214, preferably gases exiting from the zinc condenser system, and they also communicate with upper and lower conduits 216 and 218 that receive combustion-supporting gas such as air from preheating chambers 220 and 222, respectively. By this means combustion may take place alternately from the upper and lower ends of the flues, and the combustion gases exit through the idle chamber 220 or 222 so that combustion-supporting gases later passed through the chamber become preheated before use. A retort of this type is described in greater detail in United States Letters Patent No. 1,908,632.

The condensing system shown with the apparatus of Figure 4 embodies connected condensing chambers C and D for the condensation of liquid zinc and powder, respectively. Fumes from the zinc eliminating furnace are carried into the conditioning chamber B of the retort through the

flue 320, and they pass upwardly through the column of reducing or other conditioning material in a direction counter-current to the movement of the conditioning material. Heat sufficient to sustain and complete the reactions in the 5 chamber is supplied efficiently from the flues 208, but without introducing oxidizing material into the chamber or diluting the gases flowing therethrough. The conditioned gases leave chamber B through a flue 224 and then pass into the liquid 10 condenser C. Here they first flow through a section 230 in which the gases are cooled rapidly to approximately their saturation temperature by intimate contact with liquid or solid zinc. The cooling at 230 may be regulated by cooling means 15 232, so that part of the zinc content of the gases is condensed and flows downwardly over baffles or the like in contact with the rising vapors. From section 230 the gases go into a condenser 240 in which the liquid zinc is collected, and from 20 this they pass to the powder condenser D in which the residual zinc vapor is collected as powder or zinc dust. The remaining gases, containing a large proportion of carbon monoxide, leave D through a flue 242 and may be returned to the 25 retort 200 for combustion. The blue powder collected in D is continuously or intermittently returned to the upper region of the conditioning chamber B or to the cooling section 230 of condenser C, an arrangement for the latter including 30 a screw conveyor 244 being illustrated in Figure 4. If desired, preheating of the air used to combust the gases in flues 208 or for other purposes may be carried out by forcing the air through sheet metal work surrounding the condensers 35 C and D.

My improved process may be modified in many ways other than those specifically mentioned above once its freedom from limitations inherent in conventional retort smelting practice has been 40 realized. For example, an arc furnace may be used in the first or zinc eliminating operation of the process with good results, particularly when non-volatile values are to be recovered from ore in addition to volatile metals such as zinc. A great deal of freedom may also be used in the selection of apparatus, treatments and controls for the second or conditioning operation of the process and for the third operation in which the conditioned fumes are converted to desired zinciferous 45 products. 50

It will be apparent to persons skilled in the art that my improved process and apparatus are capable of practical embodiment in many different forms. I therefore desire that the invention 55 be accorded a scope sufficient to embrace equivalents, in keeping with the spirit of the specification and the requirements of the claims.

I claim:

1. In the pyrometallurgy of zinc, the process 60 which comprises releasing zinc from a reducible zinciferous charge in a chamber and supplying heat for the reduction by combustion of oxidizable material within the chamber, conducting the fumes including zinc vapor, suspended reoxidized 65 solids and combustion gases into a hot reaction zone of a separately controlled and independently heated conditioning chamber, passing the fumes in the conditioning chamber through a gas-permeable bed of hot reducing material while sup- 70 plying additional heat to reduce constituents of the fumes without externally diluting their zinc content, and condensing molten zinc from the conditioned gases in separately controlled condensing means. 75

2. In the pyrometallurgy of zinc, the process which comprises releasing zinc from a reducible zinciferous charge in a chamber and supplying heat for the reduction by combustion of oxidizable material within the chamber, conducting the fumes including zinc vapor, suspended reoxidized solids and combustion gases into a hot reaction zone of a separately controlled conditioning chamber, contacting the fumes in the conditioning chamber with hot reducing material while supplying heat to reduce constituents thereof without externally diluting the zinc content, contacting the reduced gases with condensation-promoting agents in the conditioning chamber, and condensing molten zinc from the conditioned gases in separately controlled condensing means. 5
3. In the pyrometallurgy of zinc, the process which comprises releasing zinc from a reducible zinciferous charge in a chamber and supplying heat for the reduction by combustion of oxidizable material within the chamber, conducting the fumes including zinc vapor, suspended reoxidized solids and combustion gases into a hot reaction zone of a separately controlled conditioning chamber, contacting the fumes in the conditioning chamber with hot reducing material while supplying heat to reduce constituents thereof without externally diluting the zinc content, contacting the reduced gases with an inorganic chloride in the conditioning chamber, and condensing molten zinc from the conditioned gases in separately controlled condensing means. 10
4. In the pyrometallurgy of zinc, the process which comprises releasing zinc from a reducible zinciferous charge in a chamber and supplying heat for the reduction by combustion of oxidizable material within the chamber, conducting the fumes including zinc and zinc compounds in gaseous suspension out of the liberating chamber and into a hot reaction zone of a separately controlled and independently heated conditioning chamber, passing the fumes through a porous bed of hot reducing material which moves through said zone countercurrent to the flow of the fumes and simultaneously heating said material and fumes to reducing temperatures without supplying oxidizing substances thereto, thereafter conducting the fumes out of the conditioning chamber and into cooling and condensing means and condensing metallic zinc therefrom. 15
5. The process of zinc smelting which comprises reducing zinc-bearing raw material in a first chamber to produce a mixture including zinc vapor, reoxidized zinc and gases capable of oxidizing zinc vapor before condensation thereof, flowing the mixture from the first chamber through a gas-permeable bed of hot reducing material in a second chamber and there heating the reducing material and mixture independently of said first chamber, reducing said reoxidized zinc to zinc vapor and reducing said gases to non-oxidizing form without substantial external dilution of the zinc vapor concentration of the mixture, and thereafter condensing zinc vapor in the mixture to metallic zinc in another chamber. 20
6. The process of zinc smelting which comprises reducing zinc-bearing raw material in a first chamber to produce a mixture including zinc vapor, reoxidized zinc and gases capable of oxidizing zinc vapor before condensation thereof, flowing the mixture from the first chamber through a gas permeable bed of hot reducing material in a second chamber and there heating the reducing material and mixture independently of said first chamber, reducing said reoxidized zinc to zinc vapor and reducing said gases to non-oxidizing form without substantial external dilution of the zinc vapor concentration of the mixture, and thereafter condensing zinc vapor in the mixture to metallic zinc in another chamber. 25
7. The process of zinc smelting which comprises reducing zinc-bearing raw material in a first chamber to produce a mixture including zinc vapor, suspended zinc compounds and gases capable of oxidizing zinc vapor before condensation thereof, flowing the mixture into a second chamber and into contact with reducing material hotter than the mixture, maintaining such contact for a period of at least several seconds and reducing said zinc compounds to zinc vapor and reducing said gases to non-oxidizing form without substantial external dilution of the zinc vapor concentration of the mixture, and thereafter condensing zinc vapor in the mixture to metallic zinc in another chamber. 30
8. In the pyrometallurgy of zinc, the process which comprises releasing zinc from a reducible zinciferous charge in a chamber and supplying heat for the reduction by combustion of oxidizable material within the chamber, conducting the fumes including zinc vapor, suspended reoxidized solids and combustion gases into a hot reaction zone of a separately controlled conditioning chamber, passing the fumes in the conditioning chamber through a gas-permeable bed of hot reducing material while supplying heat independently of said combustion chamber to reduce constituents of the fumes without externally diluting their zinc content, thereafter condensing molten zinc from the conditioned gases in one condenser and extracting the remaining zinc content of the residual gases as solid metallic zinc in another condenser. 35
9. In the pyrometallurgy of zinc, the process which comprises releasing zinc from a reducible zinciferous charge in a chamber and supplying heat for the reduction by combustion of oxidizable material within the chamber, conducting the fumes including zinc vapor, suspended reoxidized solids and combustion gases into a hot reaction zone of a separately controlled conditioning chamber, contacting the fumes in the conditioning chamber with hot reducing material while supplying heat to reduce constituents thereof without externally diluting the zinc content, thereafter condensing molten zinc from the conditioned gases in one condenser, extracting the remaining zinc content of the residual gases as solid metallic zinc in another condenser, and conveying solid metallic zinc from said other condenser into the conditioning chamber for redistillation to enrich the zinc vapor content of the gases passing therethrough. 40
10. The process of smelting zinc which comprises releasing zinc from a zinciferous charge in a chamber by heating the charge in the presence of reducing material, supplying part of the heat of reduction by combustion of carbon and the remainder by reoxidation of zinc vapor and carbon monoxide in the releasing chamber, passing the resulting fumes including zinc vapor, reoxidized zinc and combustion gases into a second chamber and through a gas permeable bed of hot reducing material therein, heating said reducing material and fumes independently of said first chamber, while excluding oxidizing substances, and thereby reducing reducible constituents of the fumes and conditioning the gases 45
- 75

for condensation, and thereafter condensing metallic zinc from the conditioned gases.

11. The process of smelting zinc which comprises releasing zinc from a zinciferous charge in a chamber by heating the charge in the presence of reducing material and combusting carbonaceous material, supplying most of the heat of reduction by combustion of zinc vapor and carbon monoxide generated from the charge, passing the resulting fumes including zinc vapor, reoxidized zinc and combustion gases into contact with hot reducing material while excluding oxidizing substances and thereby reducing reducible constituents thereof and conditioning the gases for condensation, and thereafter condensing metallic zinc from the conditioned gases.

12. The process of producing metallic zinc and zinc oxide as separate products from the same charge of zinciferous raw material which comprises releasing zinc from the charge by heating the charge in the presence of reducing material, supplying a substantial part of the heat of reduction by combustion of zinc vapor and carbon monoxide generated from the charge, passing the resulting fumes into a separate conditioning chamber and substantially completely reducing and conditioning them for condensation therein, condensing metallic zinc from the conditioned gases, releasing additional zinc from the charge after the reduction reaction becomes retarded by combustion of carbon in contact therewith, and burning the resulting additional fumes to collect zinc oxide.

13. The process of smelting zinc which comprises releasing zinc from a preheated zinciferous charge in a chamber by further heating the charge in the presence of reducing material, supplying part of the heat of reduction by combustion of carbon and the remainder by reoxidation of zinc vapor and carbon monoxide with preheated combustion-supporting gas in the releasing chamber, passing the resulting fumes including zinc vapor, reoxidized zinc and combustion gases into contact with hot reducing material while excluding oxidizing substances and thereby reducing reducible constituents of the fumes and conditioning the gases for condensation, and thereafter condensing metallic zinc from the conditioned gases.

14. Apparatus for the smelting of zinc comprising a furnace providing a chamber for the

generation of fumes including zinc vapor and suspended reoxidized compounds, condensing means for condensing zinc vapor to metallic zinc, separately controlled conditioning means including an enclosed bed of reducing material intermediate the furnace and condenser for receiving said fumes from the furnace, conditioning the fumes for improved condensation of metallic zinc therefrom and passing conditioned gases onward to the condenser, means for supplying heat to said material to convert the fumes to reduced condition without substantial external dilution of the zinc vapor concentration thereof, means for carrying fumes from said furnace and for introducing the same into said conditioning means in the heated portion thereof, and means for carrying conditioned gases from said conditioning means into said condensing means, said condensing means including a condenser for collecting molten zinc and another, communicating condenser for collecting zinc powder, and means for returning said powder into said conditioning means.

15. The process of zinc smelting which comprises releasing zinc from a reducible zinciferous charge in a chamber and supplying heat for the reduction by combustion of oxidizable material within the chamber, conducting the fumes including zinc and zinc compounds in gaseous suspension out of the releasing chamber and into a hot reaction zone of a separately controlled and independently heated conditioning chamber, deoxidizing a supply of carbonaceous reducing material for the conditioning chamber, maintaining a gas-permeable bed of the previously deoxidized material in said reaction zone, passing said fumes through said bed and simultaneously supplying heat to said bed and fumes, without supplying oxidizing substances thereto, to reduce the zinc compounds to zinc vapor and conditioning the fumes for condensation of metallic zinc, thereafter conducting conditioned gases out of the conditioning chamber and into cooling and condensing means and condensing metallic zinc therefrom, and from time to time removing material from said bed and adding fresh deoxidized material thereto so that the material in said bed moves in a direction counter-current to the flow of fumes therethrough.

FRANK G. BREYER. 50